

April 16, 1946.

T. A. MITCHELL

2,398,591

## METHOD OF MAKING CHROMIUM AND ITS ALLOYS

Filed Dec. 19, 1939

2 Sheets-Sheet 1



Fig. 1.

Thomas A. Mitchell Inventor

Clayton H. Jenkins

Attorney

Witness  
Herbert E. Covey

April 16, 1946.

T. A. MITCHELL

2,398,591

METHOD OF MAKING CHROMIUM AND ITS ALLOYS

Filed Dec. 19, 1939

2 Sheets-Sheet 2



Fig. 2.

Inventor

Thomas A. Mitchell

By *Clayton L. Jenkins*

Attorney

Witness  
Herbert E. Covey

## UNITED STATES PATENT OFFICE

2,398,591

## METHOD OF MAKING CHROMIUM AND ITS ALLOYS

Thomas A. Mitchell, Torrance, Calif., assignor, by mesne assignments, to Molybdenum Corporation of America, New York, N. Y., a corporation of Delaware

Application December 19, 1939, Serial No. 310,009

4 Claims. (Cl. 204—64)

This invention relates to an electrochemical method of making chromium and its alloys and more particularly to the production of such metals which have a very low content of carbon and other undesired impurities.

For various industrial purposes, such as in the production of nickel-chromium-iron electrical resistor elements as well as various other chromium alloys, it is desirable that carbon be absent or present only in a small or carefully controlled amount. Also, aluminum and other metals may be undesired elements in the production of useful steels or other alloys.

A standard method for making chromium metal involves the thermit process, wherein chromium oxide is reduced by aluminum metal; but the product contains some aluminum in spite of careful control of the reaction. Chromium may also be obtained by reduction of the oxide by means of carbon. Also a ferro-chromium alloy may be made by reduction of chromite by means of coke and a suitable flux. These reactions, however, do not result in a pure product. For example, the carbon content of ferro-chromium produced by smelting chromite may vary from 4 to 8%; and to obtain a low carbon alloy it is necessary to refine the high carbon product of the first stage, and this operation must be carefully controlled to prevent loss of the chromium metal. Other commercial processes present similar problems, wherein the operation is either expensive or does not result in a pure or satisfactory product for many desired uses.

The primary object of this invention is, therefore, to overcome such problems and to produce chromium which is substantially free from carbon and other undesired impurities.

A further object is to provide an electrochemical method for producing chromium metal and alloys thereof which is easily controlled and economically carried on and will give a product of a desired composition.

Another object is to provide a method of obtaining substantially pure chromium or an alloy thereof from impure raw materials. Other objects will be apparent in the following disclosure.

In accordance with this invention, I propose to make metallic chromium by the electro-deposition of magnesium or aluminum metal from a suitable fused bath in the presence of chromium oxide or other suitable compound, whereby the reagent metal, aluminum or magnesium, reacts as it is formed to displace the chromium from its compound and produce chromium metal. The

electrolyte is so constituted that it will dissolve compounds of the reagent metal and chromium, and an excess of the latter is maintained in the fused bath to insure reaction with all of the reagent metal deposited or tending to deposit at the cathode. Also, the bath constituents are preferably so selected and the temperature of the furnace operation so maintained that the reagent metal is deposited in a fluid condition at the cathode while the chromium or its alloys are produced in a solid non-molten condition as a sponge, tree, pellets, ingot, or in other form. The alloys of chromium with other metals, such as Fe, Ni and Cu, may be made by including one or more of the oxides of the desired alloying metals in the cell bath, and these will be reduced by the reagent metal along with the chromium. The mixture of deposited metal and solidified bath stock may be separated and the metal purified by further procedure comprising concentration of the metal and melting the concentrates as will be explained.

In the accompanying drawings:

Fig. 1 is a diagrammatic vertical section of an electrolytic cell; and

Fig. 2 is a flow diagram of the process.

The nature of the electrolyte and the constructional features of the cell are governed by the requirements for producing the reagent metal aluminum or magnesium under the above specified conditions. The electrolyte may be any suitable fused substance capable of dissolving chromium oxide as well as serving for the electrolytic production of the reagent metal, such as the fluoride of aluminum or magnesium used in suitable proportions with the fluoride of one or more metals electropositive thereto, and particularly the alkaline metals, sodium, potassium and calcium. Aluminum is molten at 660° C. and magnesium at 651° C., while chromium melts at 1615° C. The bath constituents are, therefore, so selected and the furnace cell is so operated that the bath temperature is between the melting points of chromium and the reagent metal, or above 660° C. and below 1615° C. A satisfactory electrolyte may comprise both aluminum and an alkaline metal combined with fluorine, and preferably cryolite, sodium aluminum fluoride, which melts at about 1000° C. and is a solvent for alumina, magnesia and chromium oxide. This fused bath may contain from 5 to 10% of alumina or magnesia as well as an excess of chromium oxide suspended or dissolved therein; and when subjected to a direct current electrolysis, molten aluminum or magnesium

metal tends to deposit at the cathode and there reacts in a nascent condition with the chromium oxide or other compound in solution and thus serves to build up a deposit of the metal chromium on the cathode plate.

The electrodes are so constituted and the process is so carried on as to minimize contamination of the product with carbon. Molten chromium will dissolve carbon readily; hence it is primarily desirable that the chromium product be held at a temperature below its melting point and that carbon be absent in the cathode zone. The starting cathode is a non-carbon member, such as a plate of chromium, iron or other substance. After the process has been started, the chromium deposit serves as the cathode. The anode may be made of suitable material, such as carbon, and the cell will be so operated as to maintain the anode at a distance well out of contact with the chromium deposit as it builds up.

If magnesium is used as the reagent metal in this process, magnesia may be dissolved in sodium fluoride or cryolite. The electrolysis of this bath without the oxide of chromium would result in the production of molten magnesium which would tend to float to the top of the bath and there burn when contacting with oxygen. However, the presence of chromium oxide or other compound capable of reacting instantaneously with the magnesium molecules as they are formed at the cathode reconverts that magnesium metal to the oxide where it again returns into solution for recycling in the process. Aluminum metal is similarly formed by electrolysis of the dissolved alumina, and the reaction with the chromium oxide reforms alumina which goes into solution in the bath.

The chromium oxide to be reduced may be fed as a dry powder onto the top of the fused bath, or it may be supplied to the bath as a cell lining, or preferably both methods are adopted. Care should, however, be taken to avoid contact of the chromium oxide with the carbon anode, since there may be a direct reduction of the oxide and the formation of chromium carbide. In order to form a satisfactory heat insulation for the cell walls and avoid detrimental reactions between the fused bath and the container wall, I may line the furnace with chromium oxide or a mixture of chromium oxide and the solid bath constituents. These may be used in such proportions that the bath will be replenished therefrom without change in proportions or concentration as the cell is operated. One may also introduce further charge material into the top of the furnace, and particularly to maintain a cover of undissolved and unmelted material to limit the oxidation of the anode. The chromium oxide will dissolve from this cover layer and from the lining and thus maintain a uniform concentration of chromium reagent in the bath, which is high and approaches saturation because of the continuous contact of undissolved chromium oxide with the solvent bath.

The process may be carried out in any suitable apparatus adapted for a fused bath electrolysis. This cell is preferably so made that the electrodes may be separated as the deposit is built up; and for this purpose I may so arrange the structure that the cathode and its contained cell may be moved downwardly away from an adjustable but normally stationary anode. The construction may be as shown and claimed in my copending application Serial No. 250,396 filed January 11, 1939, and which is diagrammatically 75

illustrated in the accompanying drawings as a vertical section of the cell.

The construction illustrated comprises a set of U-shaped steel rings 10 which may be made in 5 sections for the sake of replaceability, and these rings are built up one above the other to form the side wall of the cell. These side wall rings are supported on a bottom platform comprising a metal base plate 12 on which is mounted a layer 10 of insulating bricks 14 of diatomaceous earth or the like, and above which is a further layer made of suitable insulating material 16, such as asbestos. Above this is a metal plate 18 of iron, copper or other suitable non-carbon material 15 which forms the cathode. Suitable insulation 20 separates this cathode from the metal structure forming the cell chamber. Mounted above the cathode, is an anode 22 made of suitable material, such as carbon. This anode may be suitably suspended by means of a clamping ring 24 and other adjustment mechanism arranged for raising and lowering the same as required. One may use either a multiple anode, made of small cylindrical graphite rods or one may use a single large graphite body, as shown in the drawings. Power may be applied to the cell by means of a clamping ring 26 to which is attached an electrical conductor for delivering a direct current thereto. An electrical connection may be made to the cathode 20 by means of a roller 28 suitably mounted to ride against the upturned peripheral flange of the cathode plate which projects outwardly beyond the cell wall.

The fused bath may be stirred, if desired, by various types of mechanism and arrangement of the parts, such as a rotating anode or cathode. For example, I may support the metal base 12 of the cell on a lower platform 30 provided with a set of rollers 31 suitably mounted thereon and bearing against a track 32 on the underside of the plate 12. A pivot pin 33 is axially mounted in a boss on the underside of the plate 12 and supported in a boss 34 forming the center portion of the platform 30, so that the cell bottom 12 will be 40 rotatably guided by the pin. A ring gear 35 on the underside of the plate 12 is driven by means of a gear wheel 36 rotated by any suitable source of power or by hand mechanism.

The electrolytic and chemical reactions result 50 in the building up of a mass of chromium metal on the cathode plate. To prevent short circuiting by contact of this deposit with the anode, I propose to move the two electrodes away from each other periodically or continually during the process and thereby maintain proper electrolysis conditions within the cell. The anode may be made adjustable in position for this purpose as well as to feed it downwardly as oxidation consumes the rod. I prefer, however, to adjust the anode only to compensate for its being consumed and to move the cathode as the ingot builds up. This is preferably done by moving the entire cell downwardly relative to the anode. The cell including the metal cathode plate 18 and the solid deposit or ingot carried thereby may be lowered by means of a screw mechanism indicated diagrammatically by the screw 38, which is suitably mounted so that it may be operated by means of a motor or hand mechanism.

It is desirable that the chromium oxide or other reagent compound employed be fed slowly to the cell as required by exhaustion of the chromium in the solution. This may be accomplished by lining the cell wall with a material containing chromium oxide, and preferably with a mixture

of this oxide with alumina or other reagent metal oxide employed and, if desired, with solid material designed to replenish the solvent bath. Hence, the U-shaped rings 10, which are filled with a suitable insulating material 42, such as magnesia or asbestos, are provided with an innerlining 44 of these desired reagents and bath ingredients. For this purpose, the U-shaped channels of the rings 10 may be closed with plates 46 which thus form the inner wall of the cell; and this wall is arranged to carry a lining of the solid reagent material suitably cemented together and compressed in position and, if desired, baked thereon. This lining may form the sole source of the reagents and/or bath material, or it may supplement the material fed into the top of the cell.

As a specific example to further illustrate the process, I may employ for the source of raw chromium a technically pure chromic oxide containing 65 or 66% of chromium contaminated with small amounts of Fe, Si, etc. The fused bath may be sodium-aluminum-fluoride, or the mineral cryolite, herein termed an alkaline metal fluoride, to which may be added if desired, the fluorides of other metals such as aluminum, calcium and sodium for varying the melting point or for any other desired purpose. The electrolyte contains from 2 to 5% by weight of alumina dissolved therein, as well as a suitable amount of chromium oxide, such as 2 to 5% thereof. The ratio of the aluminum to the chromium may be suitably adjusted to insure efficient operation of the cell. The lining of the cell may be made of chrome brick, or it may be made up of a mixture of 50 to 60% of chromium oxide with the remainder consisting of cryolite, bonded by a small amount of molasses, pitch, tar, or other suitable material as above described. During the cell run, some of the chromium oxide may be dissolved from this lining, but the thickness of the lining is such that it remains intact to protect the steel shell of the cell. The molten cryolite or returned bath stock may be initially poured into the cell and alumina and chromium oxide added thereto. A suitable direct current is applied to the electrodes at a voltage which is ordinarily from 5 to 8 volts, and with an amperage depending upon the capacity of the cell, such as 3,000 to 10,000 amperes.

The temperature of the cell may be suitably maintained as by lowering the cell and increasing the gap between the electrodes, and thus raising the voltage. However, the reactions of aluminum or magnesium with the chromium oxide and of the evolved oxygen with the carbon of the anode are exothermic and aid in maintaining the bath temperature. The melting point of the bath will depend on the bath composition; and the mixture of fluorides will be controlled, as is well understood, to give a desired melting point. There may be some slight chemical decomposition of the bath at the operating temperatures employed, resulting in a slight loss of fluorine, and this loss may be made up by the addition of a suitable fluoride, such as cryolite or sodium, aluminum, calcium or chromium fluorides.

The reagent metal is in a molten and presumably nascent condition; and it reacts readily with the available chromium oxide and/or chromium fluoride in the solvent bath at a bath temperature below the melting point of chromium. Whether or not the chromium is momentarily molten as a result of the exothermic reaction of the aluminum and chromium oxide, it builds up as a

solid tree, sponge, contacting granules or other non-molten form of ingot. The bath is agitated by the evolving gas and the magnetic field, which aids in dissolving the solid material as it is added. The cell is continuously or periodically lowered to insure a proper spacing between the anode and the chromium deposit which grows on the cathode. As the cell is lowered, the bath stock intermingled with the chromium tree-like deposit solidifies, so that the ingot is made up of an intermixture of the bath stock and chromium metal. An analysis of the product of a typical furnace run is as follows: Cr—36% (30% metallic) Al—10%, Na—18% and F—28%.

The impurities in the metal product, such as Si and Al, may be eliminated along with the cell bath stock ingredients during a melting operation. Such a procedure may involve crushing the product and concentrating it by water classification, whereby the high density chromium metal is largely separated from the low density bath constituents. Then the concentrates to which are attached some of the solidified bath are melted in a suitable furnace which has its walls made of such material as will avoid contamination of the product. In this furnace, the bath constituents comprise principally cryolite containing dissolved alumina or magnesia and an excess of chromium oxide and/or fluorides. The melting operation thus separates the metal from the low density ingredients, which may be suitably removed. Any silicon compound that is present as an impurity will be converted to silicon fluoride, and the temperature of the bath at which chromium is molten is such that the silicon fluoride will be volatilized and thus separated from the metal. This conversion of silicon to the fluoride is caused by providing a reactive metal fluoride, such as the fluorides of alkali metal, aluminum, magnesium and chromium, and ordinarily there will be enough of the reagent in the entrapped bath stock to eliminate the silicon; but, otherwise, more of the reactive fluoride may be added for the purpose. Also, any aluminum or magnesium metal that is present as a free metal or an alloy may be removed by insuring the presence of sufficient chromium oxide or fluoride so as to convert the aluminum to the oxide or fluoride which separates from the metal as a low density slag. Magnesium is similarly separated into the slag and separated from the chromium metal. The excess of chromium oxide in the entrapped bath stock may be sufficient for the purpose of removing the reagent metal.

The accompanying flow sheet of Fig. 2 shows the preferred procedure for converting impure or pure chromium oxide into chromium metal. As there illustrated, the cell may be initially started by the use of cryolite, alumina and chromium oxide. Then when the cell run has been finished, the ingot stock comprising chromium metal with the entrapped solidified bath constituents is crushed and then ground to a fine size, such as will pass through a screen having 60 meshes per linear inch. This material is then concentrated on a standard Wilfley water classification table or by other suitable apparatus. The tailings from this table consist chiefly of the bath constituents, but with different proportions. These may be dried and then returned for use in making up the bath for a second furnace run, by being intermixed with calculated amounts of cryolite, alumina and chromium oxide as is required for the electrolyte composition. The concen-

trates on the Wilfley table are separated from the water and dried. These are then melted in a suitable type of melting pot, such as an induction furnace, where the above-described purification of the product is obtained. After separation of the slag from the metal, the mass is cooled and the resulting ingot is substantially pure chromium metal, depending upon the operation of the furnace and the nature of the reagents employed.

If it is desired to produce an alloy of chromium with other metals, such as iron, copper, nickel, cobalt and manganese, the oxides of the desired metals are introduced into the fused bath. If iron, silicon or other metal oxide is present either by intentional introduction or as an impurity in the chromium oxide or bath stock, the metallic aluminum or magnesium will reduce that oxide in the fused bath along with the reduction of the chromium oxide and thus cause both metals to appear at the cathode. The melting point of each of these metals is above that of the cryoline bath, hence each will be deposited at the cathode in a solid or non-fluid condition when a fused bath of the above described characteristics is employed. Any metal whose melting point is above that of the selected bath and whose oxide is soluble in the fused bath and is capable of being reduced by the aluminum or magnesium may be formed as an alloy with the chromium as above indicated. Hence, the claims pertaining to the formation of chromium metal are to be interpreted as covering the production of a chromium alloy where one or more other metals are formed simultaneously therewith.

It will now be appreciated, in view of the above explanation, that this process does not involve the carbon reduction of chromium oxide, and that in fact the reactions are carried on in the cathode zone away from carbon. This comprises essentially the production of a molten reagent metal by electro-chemical deposition which in turn reacts with a chromium compound in the electrolytic bath, and this reaction causes chromium to be thrown out as a metal. This process does not involve the direct electro-deposition of chromium from a chromium salt bath, but the metal is formed by reaction of a chromium compound, such as the oxide, with a more electro-positive reagent metal which is formed electrolytically in the presence of the chromium compound. It may also be observed that the sodium of the cryolite or other metal ion present which is electropositive to chromium will remain in the bath, and the electrolytic action will result only in the deposition of the reagent metal aluminum or magnesium with an evolution of oxygen at the anode. Hence, the fluoride bath serves merely as a solvent and carrier for the reagent materials.

It will now be appreciated that various modifications may be made in the process and that the compositions and the final products may be widely varied; hence, the above statements are to be considered as descriptive of the general principles of the process as well as a specific example thereof, and not as limitations on the claims appended thereto. While I have endeavored to explain the theories which are believed to underlie this process, the claims are not to be interpreted as limited to any theory or principle of operation, since it is immaterial whether or not the reagent metal is initially deposited electrolytically at the cathode or how it aids in forming the chromium deposit.

I claim:

1. The method of making chromium comprising the steps of electrolyzing in a cell between an anode and a metal cathode therebeneath a fused bath comprising a substantial amount of an oxide of a reagent metal selected from the group consisting of aluminum and magnesium dissolved in a solvent composed chiefly of a substance containing fluorine combined with aluminum and a metal selected from the group consisting of

potassium, sodium and calcium, holding the bath fused at a temperature below the melting point of chromium, progressively dissolving an excess of chromium oxide in the bath and maintaining a high concentration thereof during the electrolysis, progressively separating the anode and the associated fused bath zone from said cathode and the cell bottom and gradually forming on the cell bottom an ingot of solidified bath stock containing chromium metal which is substantially free from the reagent metal.

2. The method of making chromium comprising the steps of electrolyzing in a cell between an anode and a metal cathode located therebeneath a fused bath containing about 2 to 5% by weight of alumina dissolved in a solvent composed chiefly of a substance containing fluorine combined with aluminum and a metal selected from the group consisting of potassium, sodium and calcium, maintaining the bath fused at a temperature below the melting point of chromium, contacting the bath with solid chromium oxide and progressively dissolving said oxide and maintaining during the electrolysis a high concentration thereof approaching saturation to insure that the ultimate metal product be substantially wholly chromium, progressively separating the anode and the fused bath from the cathode and the cell bottom therebeneath, and gradually building on the cell bottom an ingot of solidified bath stock containing chromium metal which is substantially free from aluminum metal.

3. The method of making chromium comprising the steps of electrolyzing in an open cell between an anode and a metal cathode therebeneath a fused bath comprising at least 2% of alumina dissolved in a solvent composed chiefly of cryolite, holding the bath fused at a temperature below the melting point of chromium, continuously contacting the bath with solid chromium oxide and progressively feeding said oxide into the open top of the zone and maintaining during the electrolysis a high concentration of dissolved chromium oxide approaching saturation to insure that the ultimate metal product be substantially wholly chromium, progressively moving the anode and the fused bath away from said cathode and the cell bottom and gradually building on the cell bottom an ingot of solidified bath stock containing chromium metal substantially free from aluminum, and progressively supplying bath stock to maintain a predetermined volume of fused electrolyte in the cell.

4. The method according to claim 1 in which the chromium metal product and its impurities are heated with the associated bath stock containing a fluoride and chromium oxide to a temperature above the melting point of the chromium to complete the reactions and to purify the metal, after which the chromium is separated from the residue.

THOMAS A. MITCHELL.